

# United States Patent Office

**2,951,809**

Patented Sept. 6, 1960

1

2,951,809

## LUBRICATING OIL THICKENED WITH A METAL SOAP OF AN ALPHA SULFO-FATTY ACID

**John W. Nelson, Lansing, Ill., assignor to Sinclair Refining Company, New York, N.Y., a corporation of Maine**

No Drawing. Filed Mar. 1, 1955, Ser. No. 491,540.

3 Claims. (Cl. 252—33)

This invention relates to new compositions of matter and, in particular, relates to grease compositions containing, as a thickening agent, soap of an alpha-sulfo-grease forming fatty acid of at least about 12 carbon atoms per molecule.

For certain lubrication purposes which employ a lubricant of grease consistency, it is necessary for the grease to exhibit a very high dropping point. A particularly costly factor in preparing greases in general, and high dropping point greases in particular, is the soap employed as the thickener. Consequently, those in the art are constantly in search of means for reducing the amount of soap required in a grease of a given penetration, searching for alternate fatty substances which may be in greater supply or otherwise less expensive and attempting to substitute less expensive saponifying components for those presently used. These considerations are especially acute with the so-called premium greases such as those containing lithium 12-hydroxy stearate. The fatty component in such premium greases is, generally, hydrogenated castor oil or 12-hydroxy stearic acid, and continued and increased uses of these greases have made the search for substitutes for the fatty components and the lithium especially intensive.

One of the characteristics which classifies a grease as a premium grease is a high dropping point; thus, a lithium 12-hydroxy stearate grease will have a dropping point in the range of above about 400° F. and anhydrous calcium 12-hydroxy stearate grease drops at about 300° F. while ordinary calcium stearate cup greases have low dropping points on the order of 220° F. The present invention is particularly related to grease compositions evidencing high dropping points.

I have now discovered novel grease compositions which are characterized by high dropping points. These high dropping point grease compositions in general comprise a lubricating oil thickened to grease consistency with a soap of an alpha-sulfo fatty acid, preferably a saturated fatty acid, having 12 to 22 carbon atoms per molecule.

Grease compositions within the scope of the present invention include as the thickening component soaps of alpha-sulfo fatty acids. These sulfo-fatty acids include, for example, alpha-sulfo-myristic acid, alpha-sulfo stearic acid and alpha-sulfo-palmitic acids. Mixtures of the various acids within the class can also be used. Particularly desirable greases result when the fatty component employed is alpha-sulfo-stearic acid, alpha-sulfo palmitic acid, or a mixture of the alpha-sulfo stearic and palmitic acids.

The fatty material can be saponified to produce the soaps employed in my invention. In general, alkaline metals and alkaline earth metals constitute the main groups of metals which can be used. Particular components include, for example, sodium, calcium, lithium, potassium, magnesium, strontium, barium and mixtures of the foregoing, with calcium, lithium and mixtures of sodium and calcium being especially desirable. Saponifying components are used in any of the usual forms, for example, as hydroxides, oxides, carbonates and the like.

2

The resulting soaps generally constitute about 5 to 25 weight percent of the compositions and preferably about 10 to 20 percent.

5 Mineral oils or synthetic oils which normally are used in preparing grease compositions can be used in the present invention. The mineral oil fraction can be obtained from Mid-Continent, paraffinic and naphthenic crudes. In general, it is preferred that a mineral lubricating oil fraction having a viscosity within the range of about 10 50 SUS at 100° F. to 1500 SUS at 210° F. be employed. The oil fraction can be highly refined and solvent treated, if desired, by known means. Among the synthetic lubricants which can be used are polymerized olefins, alkylated aromatics, silicone polymers, polyalkylene 15 glycols and their partial or complete ethers and esters. Also I can use synthetic lubricants such as diesters of dibasic acids, e.g. di(2-ethyl hexyl) adipate and di(isooctyl) azelate, and the like.

Grease compositions of the present invention are prepared by thickening the oil fraction with soap of an alpha-sulfo fatty acid of the class described. The soaps employed can be preformed, or they can be prepared in situ. When a mono-valent saponifying component is employed, soap formation can be effected by any of the procedures known to the art. For example, both low and high temperature saponification procedures are effective as are saponification in part of or all of the oil of the final composition. On the other hand, saponification of the fatty component with a divalent material introduces a measure of flexibility permitting different soaps to be produced. Thus considering the following formula



where R is an alkyl group for instance having 12 to 20 carbon atoms it can be observed that a divalent metal can effect joinder of a plurality of molecules of the acid in a variety of ways. Examples include the following where M is a divalent metal:





The two functional groups of a single molecule also can 15 be joined as follows:



Other soaps which can be produced include polymeric soaps obtained by coupling functional groups into long chains, cross-coupling different groups, and those resulting upon the joinder of two molecules of acid by a divalent metal while neutralizing the remaining acid groups by a monovalent metal or esterifying such remaining acid groups, particularly with a lower alkyl alcohol. The various embodiments may be obtained through use of conventional blocking procedures, since the two acid groups present are of such diverse strength. Preferred calcium greases are produced by employing about 1.50 to 2.50 moles of calcium per mole of fatty component and adding the calcium incrementally, for example adding about half of the calcium slurred in starting oil, to a mixture of the acid and water and then adding the remainder of calcium after reaction has been initiated. The soap resulting appears to have the structure indicated under III above.

Premium grease compositions characteristically are substantially anhydrous, i.e., the finished greases have a water content below about 0.10 weight percent and preferably below about 0.05 weight percent. Grease compositions of the instant invention also are substantially anhydrous. Dehydration to result in this state can be accomplished in any manner but preferably by maintaining the temperature of the reaction mass, after completion of saponification, at a temperature above the boiling point of water for about 2 to 4 hours. While dehydration can be affected after finishing oil has been added, it is preferred to dehydrate prior to the addition of finishing oil in order that less material need be handled.

Grease compositions of the present invention can be formulated with a plurality of soaps. The use of a soap of an alpha-sulfo fatty acid, as noted before, results in a grease composition characterized by a high dropping point. This advantageous property can be obtained in a grease composition without the necessity of employing the alpha-sulfo soap to the exclusion of other soaps. For example, grease compositions can be made employing calcium 12-hydroxy stearate and calcium alpha-sulfo stearate with the result that a higher dropping point will be evidenced than would be evidenced by the grease containing only calcium 12-hydroxy stearate. Plural soap greases of this nature are additionally advantageous in that the stabilizing agents normally employed as in calcium containing greases need not be employed since calcium soaps of alpha-sulfo-saturated fatty acids unexpectedly exert a stabilizing effect on compositions of which they form a part. Where soaps of alpha-sulfo-saturated fatty acids are employed in conjunction with other soaps, the former generally constitutes about 5 to 75 weight percent of the total soap content.

Materials normally incorporated in greases to impart special characteristics can be added to my compositions. These include oxidation inhibitors, corrosion inhibitors, extreme pressure agents and anti-wear agents. The amount of additives added to the grease compositions usually ranges from about 0.01 weight percent up to about 10 weight percent and, in general, can be employed in any amounts desired so long as the present invention is not deleteriously affected.

10 The invention will be described further in conjunction with the following specific examples. It should be understood that the invention is not to be limited by the details disclosed in the examples.

#### EXAMPLE I

An anhydrous calcium grease was prepared as follows: 195 grams of alpha-sulfo stearic acid were treated with 22 grams of lime slurred in 400 grams of conventionally refined naphtenic type oil, having a viscosity of 200 SUS at 100° F. and 195 grams of water. This mixture was stirred in a jacketed grease kettle at room temperature for 15 minutes. Steam was gradually introduced into the jacket until the kettle contents were heated to 110° F. Then an additional 25 grams of lime slurred in 400 grams of the oil were added to the kettle and the temperature was slowly raised to 250° F. The temperature was held at about 250° F. for 2½ hours to insure essentially complete dehydration and to form the desired soap grease structure. One percent of Age-Rite Resin D-oxidation inhibitor (trimethylidihydroquinoline polymer marketed by B. F. Goodrich) was then added, finishing oil was added amounting to about 700 grams of oil and the grease was stirred until it cooled to 200° F.

Tests on the grease are as follows:

| Table I              |     |  |
|----------------------|-----|--|
| Penetration data:    |     |  |
| Unworked             | 306 |  |
| Worked, 60 strokes   | 352 |  |
| Dropping point, ° F. | 374 |  |

#### EXAMPLE II

In the preparation of a lithium alpha-sulfo stearate grease, 51 g. of lithium hydroxide mono-hydrate dissolved in 250 grams of boiling water were added to 198 grams of alpha-sulfo stearic acid dispersed in 600 grams of a conventionally refined naphtenic oil, having a viscosity of 750 SUS at 100° F. at 200° F. The temperature was raised to 338° F. during dehydration. One percent of Age-Rite Resin D oxidation inhibitor was added in conjunction with finishing oil in the usual manner, while the grease cooled to about 200° F. The grease was milled at .005" clearance in a conventional colloid mill.

Tests on this grease indicated:

| Table II             |      |  |
|----------------------|------|--|
| Penetration:         |      |  |
| Unworked             | 386  |  |
| Worked, 60 strokes   | 385  |  |
| Dropping point, ° F. | 500+ |  |

60 From the above examples it is readily apparent that greases of my invention are characterized by very high dropping points.

What is claimed is:

1. A grease composition consisting essentially of a lubricating oil base thickened with a soap of a fatty acid having twelve to twenty-two carbon atoms per molecule and a  $-\text{SO}_3\text{H}$  radical attached to the alpha carbon atom and a metal selected from the group consisting of alkali metals and alkaline earth metals.
- 65 2. The grease composition of claim 1 in which said soap is a calcium soap.
3. The grease composition of claim 1 in which said soap is a lithium soap.

## References Cited in the file of this patent

## UNITED STATES PATENTS

- 1,926,442 Gunther et al. Sept. 12, 1933  
 1,939,169 Horwitz Dec. 12, 1933  
 2,666,744 Dixon Jan. 19, 1954

## FOREIGN PATENTS

- 288,612 Great Britain Sept. 21, 1928  
 607,204 Great Britain Aug. 28, 1948

## OTHER REFERENCES

Recueil des Travaux Chimiques Des Pay-Bas, vol. 18,  
 pp. 211-214, 1899.

Chemical Technology and Analysis of Oils, Fats, and  
 Waxes, Lewkowitsch, fifth ed., vol. 1, Macmillan Co.,  
 N. Y., 1913, pp. 145 and 146.

Evidence for Alpha Sulfonation in the Reaction of  
 Palmitic Acid With Sulfur Trioxide, J. K. Weil et al.,  
 JACS 75, p. 2526 (1953).